# EUROPEAN PATENT SPECIFICATION

(11) **EP 0 055 233 B1**
(45) Date of publication and mention of the grant of the patent: **13.03.1985**
(21) Application number: 81850236.1
(22) Date of filing: 08.12.1981
(51) Int. Cl.: E01C 7/26, E01C 11/16, E01C 11/24

(54) **Composition of a surfacing mass**
Zusammensetzung einer Belagsmasse
Composition d'une masse de revêtement

(30) Priority: 19.12.1980 SE 8009020
(43) Date of publication of application: 30.06.1982
(73) Proprietor: ROCKWOOL AKTIEBOLAGET, S-541 86 Skövde (SE); SKANSKA AKTIEBOLAG, S-211 02 Malmö (SE)
(72) Inventor: Andersson, Ingmar, S-414 62 Göteborg (SE); Nilsson, Nils-Olov, S-443 00 Lerum (SE); Karlsson, Elis, S-532 02 Axvall (SE); Sandberg, Ulrik, D-541 31 Skövde (SE)
(74) Representative: Avellan-Hultman, Olle

## Description

The present invention relates to a composition of a surfacing mass for streets, roads, parking places etc. having a draining activity and comprising a mixture of a stone material and asphalt, according to the preamble of claim 1. The invention also relates to a method of manufacturing such surfacing mass.

The present general high speeds of road vehicles have caused a demand that rain water quickly disappears from the surface of the road. The most serious consequences of water on the road surface is water planing, whereby the tire is separated from the road surface by a film of water. Water planing may appear already at relatively low speeds and is considered to be the reason for numerous serious traffic accidents. Also in other ways water on the road surface may cause difficulties for instance in that the vehicle tires splashes water thereby impairing the visibility.

A reasonably quick run off of water may be obtained when the road is formed cambered but depending on wear, especially when using tire pegs, and depending on the packing and deformation that heavy traffic causes depressed wheel tracks appear in which water may be collected in spite of the fact that the road is cambered.

The water filled wheeltracks of course increase the risk of water planing and may upon sudden temperature changes in the winter be transformed to dangerous ice areas. Another problem which in particular has appeared when setting up large asphalt or concrete surface parking places is that such surface coverings involve disturbances in the natural percolation or the natural drainings. The rain water can not penetrate the tight coverings and is not returned as subsoil water but is collected as surface water which in turn must be drained and often also must be cleaned. Even if there is normally no problems involved in water planing at parking places, such places ought to be as waterfree as possible since people have to walk there.

One solution of the said problems has been to provide the water surface, the parking place etc. with a covering having a large amount of cavities so that the covering thereby becomes water pervious. In such surfacing masses which comprises a stone material having asphalt as a binder and which consequently comprises a portion of coarse material and a portion of fine material the surfacing mass has been given a low amount of fine material so that the masses obtain a large number of communicating cavities. Since thereby only a part of the volume of the cavities or the stone material is filled with asphalt or any other fine material there is a remainder of cavity volume in the ready surfacing mass. For well drained masses such a cavity volume is at least 15-25% which amount should be compared with normal non-drained .surfacing masses which according to actual (Swedish stipulations) should have a cavity volume of 2-6%.

The experiences of such so called open grades asphalt friction courses have shown that such masses, apart from the said draining property, also have other good properties. Among such properties is noted that the masses in combination with rubber tires give a high friction and a silent run. Road markings have better visibility and have a longer lifetime against wear. Especially at nights wet surfac- ings of this type give less reflexes than the conventional tight surfaces.

Open grades asphalt friction courses, however, are disadvantageous in some respect. Depending on its porosity open grades asphalt friction courses cannot be provided anywhere, for instance not on cracked substrates. When laying such surface coverings also particular rules must be fulfilled. At places where so called open grades asphalt friction courses have been applied, however, generally positive experiences have been met with.

The manufacture of such drained surfacing masses, however, involve large problems. At normal temperature for mixing the stone mass and the asphalt, which for asphalt having the temperature designation A-120 or A-135 according to the ASTM standard (at 500 cSt) is 150-160°C the asphalt flows off the stone since there is not sufficient amount of fine grain material for keeping the thin fluid asphalt. Such flow off of the asphalt sometimes leads to "degraining" or segregation at handling, transport and surface covering since the coarse grains are separated from fine grains thereby causing so called stone loss in the ready surface covering, all depending of the fact that the surfacing mass cannot be made to contain sufficient amount of asphalt.

For solving this problem attempts have been made to make the mixture at lower temperatures. It has shown that such a little run off of asphalt from the stone material is obtained at a mixing temperature of 115-120°C that drained surfacing masses can be made which having such high amount of asphalt that there is no substantial degraining or no substantial stone loss. The low mixing temperature, however, has added new problems. For eliminating the influence of remaining moisture in the stone material which prevents the asphalt from wetting the stone surfaces it is among other things necessary to add some wetting improving means. For this purpose certain amines, for instance an alcyle amine like the amine marketed under the trade mark "Lilamin VP75" used to be added in an amount of about 0,4% as calculated on the amount of asphalt. The amines, however, give an upleasent smell, both when manufacturing the asphalt in the asphalt mill and when laying the surfacing masses.

Also hydrated lime has been used in an amount of for instance 1,5% as calculated on the stone material for eliminating the remaining moisture of the stone material. Since, however, both amines and hydrated lime are classified as dangerous substances particular measurements of safety must be considered when using such substances. The lower mixing temperature for asphalt and stone material also necessitates a time consuming and expensive readjustment of the asphalt mill. Also the surfacing mass mixed at low temperature shows an unfavourable tendency to post packing or post compressing what especially in summers at heavy traffic load cause relatively strong wheel tracks. Also the post packed part of the surfacing gets a tightening especially of the surface to the effect that the draining property of the surfacing is reduced just on places where such property would be of best need.

It has previously been suggested to increase the viscosity of the asphalt binder by adding a fine grain filler material. According to the Swedish Patent 211,163 an especially large effect per part of weight is obtained if the filler material is a mineral fiber having a diameter of 5-15 um. If the viscosity is increased by adding a filler material there is a less run off of asphalt from the stone material, but it has appeared self explanatory to the expert that an increase of viscosity by admixing a filler material would give the same post-packing problems as an increase of viscosity by lowering the temperature. The method suggested in the said patent therefore has not been used to any substantial extent.

Now it has surprisingly shown that both of the above mentioned problems may be solved by using mineral fibres of special dimensions according to the characterizing portion of claim 1, viz. the problem of avoiding asphalt run off from the stone material and to avoid the troublesome post-packing problem. This is possible even when mixing the surfacing mass at the normal asphalt mixing temperatures of 150-160°C. It has shown that this is possible if a sufficient large amount of fibre material having sufficiently thin fibres is admixed in the asphalt phase and the mixing is made at the normal asphalt mixing temperature of 150-160°C. The adhesion between asphalt and stone material is not influenced by the admixing of fibres and this means that no particular adhesion improving substances have to be added. Since the mixing temperature is kept at normal level no time consuming and complicated readjustments have to be made in the asphalt mill and it has shown that the surfacing mass of the above mentioned type gives fully acceptable values as concerning the post packing or post compressing. Thereby the above mentioned problem of tightening of the covering surface and thereby the reduced draining property depending on the pressure from the vehicle tires are eliminated or substantially reduced.

Apart from the demand that the added filler material should have a predetermined small average diameter it is also a need that the fibres should be resistant and should not become softened at the actual mixing temperature. It has shown that particularly good results are obtained by means of mineral fibres having an average fibre diameter which is less than 5 pm and more than 1 µm.

Tests have shown that fibres which are coarser than 5 _{µ}rn do not have a sufficient viscosity increasing effect and obviously also not reinforcing effect to the binder film. The latter disadvantage possibly may be explained in that the fibres to a large extent tend to orientate parallelly to the stone and thereby also to the plane of the binder film.

If on the other hand a less average fiber diameter than 1 µm is used the viscosity is indeed influenced, but the reinforcing effect is bad. Obviously there is an area of 1-5 pm for the average fibre diameter which seems to be an optimum.

It has also shown advantageous that the mineral fibres are made to appear separated from the other in the asphalt phase so as not to form knots or tots. The formation of such knots or tots may be prevented by admixing the fibres in a suitable way and by pretreating the fibres with some substance which simplifies for the asphalt to wet the fibre surface. For this purpose wetting agents known per se like cationic tensides may be used. The asphalt wetting of the fibre surfaces also may be facilitated in that all moisture is removed from the fibres by drying the fibres before adding the fibres to the asphalt mass.

The admixing of the fibre material preferably is made into the asphalt before the stone material is added. A good and tot free admixing may be obtained if the asphalt is heated to a temperature of for instance 20-40°C over the normal temperature for admixing the stone material in connection to the admixing of the fibres, and in that the asphalt-fibre mixture is cooled to the said normal stone material admixing temperature before the stone material is added. The said temporary temperature increase gives a particularly good effect in the case that the wetability between asphalt and fibres is improved in that the fibre surfaces are treated with some wetting agent or in that the fibres are dried. Depending on the risk of fire at the increased temperature the process ought to be accomplished in closed state.

To summarize the invention relates to a composition of a surfacing mass based on asphalt and a method of manufacturing such a surfacing mass which has draining properties and which comprises a stone material having a low amount of fine material and having asphalt as a binder. In the method according to the invention the admixing of stone material is made at a temperature for the asphalt of preferably 150-160°C and in the presence of 0,5-20% by weight as calculated on the amount of asphalt of a fibreous material which is not solved or softened in the asphalt. Tests have proved that a sufficient effect for the method to be of technical-economical interest is not obtained if the fibres are present in an amount of less than 0,5%, that is such low amount of fibres cannot justify the admixing costs and the fibre costs. Further tests have shown that higher fibre amounts than 20% do not give improved properties corresponding to the increased costs for the increased amount of fibres.

In the following some examples of the invention will be given. It is, however, to be understood that the examples are only of illustrating nature.

### Example 1

In a batch mixing mill for asphalt masses 3,144 kg of a stone material having the following average size composition was introduced:

The stone material was heated to 160°C. 160 kg asphalt having the denomination temperature of A-135 according to ASTM standard was added at a temperature of 160°C by means of 40 nozzles. Shortly before the introduction of the asphalt the stone material was mixed with 32 kg mineral fibres of the type manufactured by Rockwool Aktiebolaget and marketed under the registered trade mark Inorphil 057. "Inorphil 057" is a mineral fibre material having an average fibre diameter of about 3 pm and in which the main part of the fibres has a fibre diameter within the area of 1-5 µm. For characterizing the length of the fibres there are no acceptable direct methods. Instead thereof preferably the so called thickening number (n_{f}) is measured, which number is

in which 17 is the viscosity of a slurry of 0,5 g dry fibres in 200 ml ethylene glycol at 20°C and in which 77. is the viscosity of the same ethylene glycol without fibres likewise at 20°C and measured by means of the same measuring equipment, which is a Brookfield viscosimeter having a spindle LV1 or corresponding. For fibres of the type marketed by Rockwool Aktiebolaget under the trade mark "Inorphil 057" the thickening number is 1,8-6,0.

After the mixing was finished the mass was taken out and the run off of asphalt from the stone material was observed and judged. The judging which was made according to the following scale showed to have a clearly acceptable result, point B in the following. The post packing was judged to below for a draining surfacing mass of this type and showed to correspond to normal post packing for conventional non-draining surfacing masses. The run off of asphalt from the stone material was determined in the following way:
With a minimum of handling 100 g of the mass was taken out and was placed on a circular heat resistant glass plate having a diameter of 203 mm. The glass plate was placed in a heat box at 160°C and was observed from underneath for 60 minutes. The following judging scale was used:
   A Asphalt only in the contact point between stone and glass;
   B Small asphalt dabs in each contact point;
   C Several large asphalt dabs in some of the contact points;
   D Large asphalt dabs in each contact point.

### Examples 2-5

The same method was used as in example 1 with the difference that 16, 6,4, 1,3 and 0,65 kg mineral fibres respectively of the type "Inorphil 057" was added. The result is shown in the table underneath. It is evident that a less addition of mineral fibres than about 0,5% gave an unsatisfactory run off and in addition thereto a non-satisfactory value of post packing of the ready asphalt mass.

### Example 6

In a batch mixing mill for asphalt masses 3,158 kg of a stone material having the same distribution of size as in example 1 was introduced. The stone material was heated to 160°C. Separately and concurrently therewith 166 kg asphalt having the denomination temperature A-135 was heated to 160°C and to the heated asphalt was added 16 kg mineral fibres of the same type as in example 1. The asphalt and the mineral fibres was mixed and was added at maintained temperature to the heated stone material, and all ingredients were mixed.

The run off was observed and judged in the same way as in example 1. In spite of the less amount of mineral fibres the surfacing mass proved to have the same run off the post packing properties as in example 1.

### Example 7-8

The same method was repeated as in example 6 with the difference that instead of 6,4 kg mineral fibres was now added 1,3 and 0,65 kg respectively of mineral fibres of the same type as in example 6. The result is shown in the following table. It is evident that also in this case a less. amount of mineral fibres than 0,5% gives an unsatisfactory result.

### Example 9

The method according to example 6 was repeated but with the difference that the asphalt was heated to 190°C before the admixing of the mineral fibre and in this case mineral fibres of the type "Inorphil 057" was added in the same amount as in example 6. The mixture of asphalt and mineral fibre was cooled to 160°C before the mixing together with the stone material.

The result is shown in the table.

### Examples 10-11

The method according to example 9 was repeated, but in this case was added 1,3 and 0,65 kg mineral fibres respectively. The result shown in the table confirms that an amount of mineral fibres of less than 0,5% as calculated on the amount of asphalt gives an unsatisfactory result.

The run off was observed and judged in the same way as in the previous examples, and the surfacing mass showed to have the same good properties as in the previous examples.

Depending on the extra heating of the asphalt mass in connection to the admixing of the mineral fibres the amount of mineral fibres consequently could be further reduced without obtaining impaired properties of run off and post packing.

### Example 12

For a comparing analyzis the method of claims 1-5 was repeated, but instead of the mineral fibres "Inorphil 057" mineral fibres having an average fibre diameter of 6-8 µm was added.

The run off and post-packing properties were observed in the same way as in the previous examples. The coarse fibre portion was manufactured by separating away all unfibrated material from coarse fibre basalt wool and a part of the fibres less than 5 µm.

The run off showed to be larger than in examples 1-5 and was judged to be non-acceptable (D), see the following table.

### Example 13

The method according to claim 1 was repeated but with a mineral fibre material the average fibre diameter of which was less than 1 µm. The run off and post packing properties were observed, and the run off proved to be non-acceptable (E) and the post packing properties were essentially higher than in examples 1-5.

The following table clearly proves the connection between the fibre size and the run off appearance of the asphalt-stone-fibre material and thereby also the connection between the fibre size and the porosity and the water- perviosity of the ready surfacing mass. It is thus clearly evident that fibres having a larger diameter than about 5 µm give an impaired run off value than fibres within the area of 1-5 µm.

## Claims

1. Composition of a surfacing mass for streets, roads, parking places etc. having a draining activity and comprising a mixture of a stone material and asphalt, the stone material having a small portion of fine material, and the stone-asphalt mixture comprising a small amount of fibres characterized in that the average fibre diameter is more than 1 and less than 5 um.

2. Composition of a surfacing mass according to claim 1, characterized in that the stone material mainly comprises stone particles having an average diameter of between 2 and 12 mm, and in that about 50% of the stone material has an average particle size of 8-12 mm, and in that the amount of fibres is about 0,5-20% by weight of the asphalt mass.

3. Composition of a surfacing mass according to claim 1 or 2, characterized in that the fibre material is treated with a wetting agent, for instance a cationic tenside.

4. Method of manufacturing a surfacing mass according to any of the preceding claims for streets, roads, parking places etc. having draining activity and comprising a mixture of stone material and asphalt, characterized in that a stone material having a little portion of fine material is mixed with an asphalt phase at a temperature of 140-170°C or preferably 150-160°C in the presence of 0,5-20% by weight, as calculated of the amount of asphalt, of a fibre material of a type which is not solved or softened in the asphalt and which has an average fibre diameter of less than 5 _{fl}m and more than 1 µm and which is substantially evenly distributed in the asphalt phase with the fibres separated from each other.

5. Method according to claim 4, characterized in that the fibre material is admixed in the asphalt before the asphalt is mixed with the stone material.

6. A method according to claim 4 or 5, characterized in that the fibre material is treated with a wetting agent, for instance a cationic tenside before the fibre material is added to the asphalt phase.

7. Method according to any of claims 4-6, characterized in that the fibre material is completely dried before being admixed in the asphalt phase.

8. Method according to claim 6, characterized in that the asphalt is heated to a temperature of about 20-40°C over the mixing temperature for asphalt and stone material before the fibre material is added to the asphalt, and in that the mixture of asphalt and fibre material is cooled to the temperature of the stone material and is mixed with the stone material.

## Patentansprüche

1. Zusammensetzung einer eine Drainagewirkung entfaltenden Belagsmasse für Straßen, Wege, Parkplätze u. dgl., die eine Mischung aus Steinmaterial und Asphalt enthält, wobei das Steinmaterial einen geringen Anteil feinen Materials und die Stein-Asphaltmischung einen geringen Anteil von Fasern haben, dadurch gekennzeichnet, daß der mittlere Faserdurchmesser größer als 1 ,um und kleiner als 5 ym ist.

2. Zusammensetzung einer Belagsmasse nach Anspruch 1, dadurch gekennzeichnet, daß das Steinmaterial hauptsächlich Steinpartikel mit einem mittleren Durchmesser zwischen 2 und 12 mm enthält und daß etwa 50 % des Steinmaterials eine mittlere Teilchengröße von 8 bis 12 mm aufweist und daß der Faseranteil 0,5 bis 20 Gew.% der Asphaltmasse beträgt.

3. Zusammensetzung einer Belagsmasse nach Anspruch 1 oder 2, dadurch gekennzeichnet, daß das Fasermaterial mit einem Netzmittel, z. B. einem kationischen Tensid, behandelt ist.

4. Verfahren zur Herstellung einer eine Drainagewirkung entfaltenden Belagsmasse für Straßen, Wege, Parkplätze u. dgl., die eine Mischung aus Steinmaterial und Asphalt enthält, nach einem der vorgehenden Ansprüch, dadurch gekennzeichnet, daß ein einen geringen Anteil feinen Materials enthaltendes Steinmaterial mit einer Asphaltphase be 140-170°C, insebesondere bei 150-160°C, im Beisein von 0,5-20 Gew.%, bezogen auf den Asphaltanteil eines Fasermaterialsvermischt wird, wobei das Fasermaterial von solcher Art ist, daß es nicht im Asphalt gelöst oder erweicht wird und die Fasern einen mittleren Faserdurchmesser von weniger als 5 um und mehr als 1 µ aufweisen und diese Fasern weitgehend gleichmäßig in der Asphaltphase verteilt und voneinander getrennte sind.

5. Verfahren nach Anspruch 4, dadurch gekennzeichnet, daß das Fasermaterial dem Asphalt zugemischt wird, bevor der Asphalt mit dem Steinmaterial gemischt wird.

6. Verfahren nach Anspruch 4 oder 5, dadurch gekennzeichnet, daß das Fasermaterial mit einem Netzmittel, z. B. einem kationischen Tensid, behandelt wird, bevor es der Asphaltphase zugesetzt wird.

7. Verfahren nach einem der Ansprüche 4 bis 6, dadurch gekennzeichnet, daß das Fasermaterial vollständig getrocknet wird, bevor es der Asphaltphase zugemischt wird.

8. Verfahren nach Anspruch 6, dadurch gekennzeichnet, daß der Asphalt auf eine Temperatur erhitzt wird, die 20-40°C oberhalb der Mischungstemperatur für den Asphalt und das Steinmaterial liegt, bevor das Fasermaterial dem Asphalt zugesetzt wird und daß die Mischung Asphalt/Fasermaterial auf die Temperatur des Steinmaterials abgekühlt und mit dem Steinmaterial gemischt wird.

## Revendications

1. Composition de revêtement pour rues, routes, aires de stationnement, etc., ayant une activité de drainage et comprenant un mélange de pierre et de bitume, la pierre renfermant une petite proportion de fines et le mélange pierre- bitume comprenant une petite quantité de fibres, caractérisée en ce que le diamètre moyen des fibres est supérieur à 1 µm et inférieur à 5 µm.

2. Composition de revêtement suivant la revendication 1, caractérisée en ce que la pierre est principalement formée d'éléments ayant un diamètre moyen compris entre 2 et 12 mm et en ce qu'environ 50 % de la pierre ont un diamètre élémentaire moyen de 8 à 12 mm, et en .ce que la quantité de fibres est d'environ 0,5 à 20 % en poids de la masse bitumineuse.

3. Composition de revêtement suivant la revendication 1 ou 2, caractérisée en ce que la matière fibreuse est traitée avec un agent mouillant, par example avec un agent tensioactif cationique.

4. Procédé de production d'un revêtement suivant l'une quelconque des revendications précédentes pour des rues, des routes, des aires de stationnement etc., ayant une activité de drainage et comprenant un mélange de pierre et de bitume, caractérisé en ce que de la pierre refermant une faible proportion de fines est mélangée avec une phase bitumineuse à une température de 140 à 17µ°C ou notamment de 150 à 160°C en présence de 0,5 à 20 % en poids, exprimé, par rapport à la quantité de bitume, d'une matière fibreuse d'un type qui ne se dissout pas ou ne se ramollit pas dans le bitume et dont les fibres ont un diamètre moyen de moins de 5 µm et de plus de 1 µm et qui se distribue uniformément dans la phase bitumineuse, avec séparation des fibres les unes des autres.

5. Procédé suivant la revendication 4, caractérisé en ce que la matière fibreuse est incorporée au bitume avant que ce dernier no soit mélangé avec la pierre.

6. Procédé suivant la revendication 4 ou 5, caractérisé en ce que la matière fibreuse est traitée avec un agent mouillant, par exemple un agent tensioactif cationique, avant qu'elle ne soit ajoutée à la phase bitumineuse.

7. Procédé suivant l'une quelconque des revendications 4 à 6, caractérisé en ce que la matière fibreuse est complètement séchée avant d'être incorporée à la phase bitumineuse.

8. Procédé suivant la revendication 6, caractérisé en ce que le bitume est chauffé à une température d'environ 20 à 40°C au-delà de la température de mélange du bitume et de la pierre avant que la matière fibreuse no soit ajoutée au bitume, et en ce que le mélange de bitume et de matière fibreuse est refroidi à la température de la pierre et est mélangé avec cette dernière.
